

Sept. 24, 1935.

M. M. AUSTIN

2,015,509

HARD TANTALUM AND METHOD OF HARDENING

Filed Feb. 28, 1931

Fig. 1.



Inventor:  
Miner M. Austin  
By William E. Bradbury,  
McCaleb & Hinkle,  
Attns.

## UNITED STATES PATENT OFFICE

2,015,509

HARD TANTALUM AND METHOD OF  
HARDENINGMiner M. Austin, Highland Park, Ill., assignor to  
Fansteel Products Company, Inc., North Chi-  
cago, Ill., a corporation of New York

Application February 28, 1931, Serial No. 519,177

10 Claims. (Cl. 148—16)

This invention relates in general to hardened metals and has more particular reference to hardened tantalum and a method of hardening the same.

5 A primary object of the present invention is the provision and production of hardened tantalum and articles thereof.

An important object of the invention is to provide a novel method of controlledly hardening 10 tantalum and tantalum articles.

Another important object of the invention is to treat a degasified refractory metal in a reduced atmosphere to harden the refractory metal and to control such hardening by controlling the 15 absorption of the air by the refractory metal.

A further important object of the invention is the provision of case hardened tantalum and tantalum articles, and a novel method of producing such tantalum or articles having the 20 desired hardness.

Other objects and advantages of the invention will be apparent from the following description and from the accompanying drawing, in which similar characters of reference indicate similar 25 parts throughout the several views.

In the drawing

Fig. 1 is a diagrammatic view of apparatus suitable for treating the refractory metal and articles thereof in accordance with the invention; 30 and

Fig. 2 is a transverse sectional view of a heating element suitable for use in my novel method and showing a refractory metal in place for the hardening operation.

35 There are various uses to which a substantially non-corrosive and wear resistant hard metal may advantageously be put. For example, spinnerets used in the manufacture of artificial silk or rayon, which are provided with fine circular openings or apertures. These spinnerets are subjected in use to acid solutions, and must be non-corrosive or acid resisting, hard and durable, or wear resistant, because if the openings are slightly distorted or flat, the rayon produced will be of an inferior 40 quality and will consequently cause a pecuniary loss when sold.

Other uses of a hard, non-corrosive and durable metal will be apparent, the foregoing embodiment being recited merely by way of example.

50 For instance, turbine blades, chemical and electro-chemical apparatus, and other heavy duty articles which in their use are subject to wear or corrosive atmospheres.

The properties of tantalum have already caused 55 this material to be a favorite for such uses, but

in many instances, it is desirable to have a material with the non-corrosive or acid resisting and hard qualities of tantalum, together with a greater degree of hardness, durability or wear resisting qualities and workability.

It has been suggested to provide a material harder than tantalum and with some of its properties, by alloying tantalum with a harder material, such as tungsten, and by alternately heating and hammering tantalum. The tantalum-tungsten alloy is objectionable for such uses, because the degree of hardness is not readily controllable, and the resulting properties of such an alloy are not altogether desirable. Moreover, such an alloy is expensive to produce, and does not possess 10 the degree of hardness required for such uses, and is not readily workable.

It is conceivable that the method of alternately heating and hammering tantalum might produce hardened tantalum, but such a method does not 20 readily adapt itself to controlledly hardening tantalum, and must be painstakingly carried out, the method being highly impractical and subject to many other limitations.

By an exhaustive study of the properties of 25 tantalum and by the application of prior art methods of hardening other metals, three methods readily suggest themselves as being practical and possibly successful. These three methods are heating the tantalum in air at atmospheric 30 pressure, heating and quenching the tantalum, and heating tantalum in an atmosphere of a gas which tends to combine with tantalum to produce a hard composition.

I have tried these three methods and found that 35 no useful hardness of tantalum can thereby be obtained, but that a vigorous reaction occurs at the surface of the tantalum and very little penetration of gases to the interior of the tantalum results. Moreover, such methods result in dis- 40 coloration and rotten metal.

Briefly, the present invention contemplates a novel method for overcoming the foregoing objections and producing tantalum or articles having a varying degree of hardness from the outer 45 surface inwardly, a degree of hardness uniformly distributed throughout the section of the tantalum or tantalum article, or a hardened case on the tantalum or an article made therefrom. In order to accomplish the foregoing objects, I heat 50 tantalum or tantalum objects in a reduced pressure, to a temperature at which the gases occluded by the metal are freed, and separate or pump such gases from the container in which the tantalum is heated. This degasified tantalum is 55

5 maintained at the degasification temperature in a reduced pressure and measured quantities of air are successively admitted to the tantalum heated in a reduced pressure, and are absorbed uniformly by the surface of the tantalum. Further 10 heating of the tantalum carrying at its surface this absorbed air, operates to diffuse the air in the body of the material and to diffuse or distribute, as it were, the hardness of the material 15 from the surface inwardly thereof. The degree of hardness is apparently determined by the amount or quantity of air absorbed by the tantalum or tantalum article, and the diffusion of the air throughout the tantalum body and the 20 degree of hardness may therefore be controlled by the amount or quantity of air admitted to the tantalum heated in a reduced pressure, and the control of the time during which the tantalum 25 is heated.

20 It will of course be apparent that a hardened case may be formed on the tantalum or tantalum articles by admitting the desired amount of air and continuing the heating of the tantalum until the air is absorbed by the surface of the tantalum, 25 and this hardness may be made to vary from the surface of the tantalum body inwardly thereof until the air is uniformly distributed throughout the section, at which time the material is uniformly hard, by controlling the time during which 30 the tantalum is heated.

30 While I do not wish to limit my invention to any particular apparatus for accomplishing the novel results, I have illustrated by way of example in the drawing, suitable devices for hardening tantalum. This apparatus comprises any suitable heating unit or furnace capable of developing the desired temperatures and of providing a heating vacuum chamber, such, for example as a quartz tube 5, closed at each end by 35 means of rubber stoppers or caps 6 and provided with a source of heat which I have illustrated as an external coil 7 encircling the quartz tube 5 and connected by means of conductors 8 to a suitable source of electrical potential, not shown.

40 The electrical energy supplied to the coil 7 may be controlled by any suitable switch 9, as shown in the drawing.

45 A frame, receptacle, or holder 11 of any suitable metal capable of withstanding the temperature developed within the quartz tube 5, is provided for carrying the tantalum or tantalum articles to be treated. This holder or receptacle 11 is preferably of tantalum or any other suitable high-melting point metal or alloy and is illustrated as 50 a cylinder carrying tantalum strips or articles 12, as shown in Fig. 2, or the tantalum cylinder may be provided with a plurality of apertures 13 as shown in Fig. 1 for carrying a plurality of spinnerets or other tantalum articles 14.

55 60 This holder or receptacle carrying the tantalum or articles to be hardened, is inserted in the tube 5 and may be supported therein by any suitable means, such as brackets 15 at each end of the tantalum receptacle. Where the stoppers or caps 6 are constructed of an inflammable material, they may be protected from the heat within the quartz tube 5 by means of heat baffles or reflectors 16 positioned at each end of the quartz tube 5 between the stoppers or caps 6, and the corresponding 65 ends of the receptacle or holder 11.

70 The interior of the quartz tube 5 is connected by means of a tube 17 or any other suitable connector passing through one of the stoppers 6 to any suitable vacuum pump, not shown, for the 75 purpose of reducing or exhausting the atmosphere

within the tube 5. The action of the vacuum pump on the interior of the tube 5 is controlled by a valve 18, which at the beginning of the operation, is open, and the pump is operated to reduce the pressure within the tube 5 to about 1 millimeter of mercury, which reduced pressure is maintained until the tantalum or tantalum articles are heated to from 1200° to 1400° C. by means of the heating coil 7. This pressure may be indicated by any suitable pressure indicating mechanism, such as a manometer 19 connected to the tube 17, as shown in Fig. 1, and the heating of the tantalum and tantalum articles is continued until the manometer 19 indicates that substantially all of the occluded gases have been 15 driven out of the tantalum or articles being heated. When such a condition is indicated, the valve 18 is closed, disconnecting the pump from the tube 5, and a valve 21 communicating with a measuring flask 22 at one end, and with atmosphere at 20 the other is opened to admit air at atmospheric pressure to the measuring flask 22. The valve 21 is then closed and a valve 23 is opened to admit the air in the measuring flask to the tube 17 to which the flask 22 is connected by means of a 25 tube 24 for supplying air to the interior of the quartz tube 5.

20 Thus, a measured amount or quantity of air is supplied to the quartz tube 5 and the increased pressure within the tube will be indicated by the 30 manometer 19. The heating of the tantalum or tantalum articles in the quartz tube 5 is continued until the manometer 19 indicates a return of the initial reduced pressure, whereupon the valve 23 is closed and the valve 21 opened to admit a 35 further supply of air to the measuring flask 22, which may subsequently be supplied to the interior of the quartz tube 5, as described above.

35 The amount of air required to produce the desired degree of hardness, may be determined by 40 experiment and upon supplying such amount to the tantalum within the quartz tube, the valve 23 may be closed and the heating continued to properly diffuse the gas carried by the surface of the tantalum or tantalum article inwardly of the 45 tantalum to provide the hardness properties desired.

40 It will of course, be apparent that the measuring flask 22 communicating with the interior of the quartz tube 5 and with atmosphere, merely 50 diagrammatically illustrates one means by which it is possible to supply and control the supply of air to be absorbed by the tantalum, it being here contemplated as within the scope of the present invention to use any suitable controllable and 55 measurable source of air supply.

45 As already mentioned, the amount of air absorbed by the tantalum or articles made therefrom to produce the desired degree of hardness, may be determined by experiment, and I have 60 found that, in hardening a plurality of spinnerets arranged as shown in Fig. 1 within a quartz tube having a volume of about 2750 cubic centimeters, air may be admitted in 125 cubic centimeter portions or quantities from time to time as the spinnerets 65 absorb these portions of air for a period of about one hour during which time approximately 1000 cubic centimeters of air was absorbed by the spinnerets.

55 I have found that about 1000 cubic centimeters 70 of air per 1000 grams of tantalum will produce a marked springiness if the heating is continued until the air is diffused throughout the metal, and that in such proportions a file hard surface or case is formed on the tantalum if the diffusion 75

is not caused by further heating of the tantalum. Moderate hardening of either the surface or the body may be obtained by reducing these proportions and greater hardening may be obtained by increasing such proportions. The metal or articles, when so treated, take on a bright, metallic appearance, and if the gassing were moderate, the metal could be worked by rolling or swaging to produce additional work hardness or to produce desirable shapes.

Illustrative of the advantages of tantalum when so hardened, I have found that tantalum spinnerets may be provided with a suitable hardness to protect the fine openings therein and non-  
corrosive qualities which promote durability of the spinnerets in service and obviate the necessity of frequently replacing such spinnerets.

While I have described the novel method as applied to tantalum, it is understood that other similar metals, such, for example, as columbium, may be treated in the same manner, and that possibly other gases, such as nitrogen, hydrogen or pure oxygen, may be substituted for air, and that I am not limited to the details as hereinabove set forth, except as defined by the following claims.

I claim:

1. A method of gas hardening a hard refractory metal from the group consisting of tantalum and columbium, by causing the hard refractory metal to absorb a hardening constituent of air, which comprises degasifying said refractory metal by heating it at a reduced pressure to from 1200° to 1400° C., supplying air to said hard refractory metal, heating said hard refractory metal to the absorbing temperature for a hardening constituent of air whereby to cause absorption thereof by said hard refractory metal, and continuing such heating of such hard refractory metal to cause said constituent of air to penetrate into said hard refractory metal whereby to harden it throughout.

2. A method of gas hardening tantalum, which comprises degasifying said tantalum by heating it at a reduced pressure to from 1200° to 1400° C., supplying air to said tantalum, heating said tantalum to the gas absorbing temperature for air whereby to cause absorption of the air by said tantalum, and continuing such heating of said tantalum to cause the absorbed air to penetrate into the tantalum whereby to harden it throughout.

3. A method of gas hardening a hard refractory metal from the group consisting of tantalum and columbium by causing it to absorb a hardening constituent of air, which comprises heating said hard refractory metal at a reduced pressure to from 1200° to 1400° C., whereby to degasify said hard refractory metal, successively supplying predetermined quantities of air to said hard refractory metal while heating the hard refractory metal to the absorbing temperature for the hardening constituent of air until said hard refractory metal absorbs it in the proportion of about 100 cubic centimeters of the constituent of air to 100 grams of said hard refractory metal, and continuing the heating of said hard refractory metal with said constituent of air absorbed thereby to diffuse the absorbed constituent of air throughout said hard refractory metal.

4. A method of gas hardening tantalum, which comprises heating said tantalum at a reduced pressure to from 1200° to 1400° C., whereby to degasify said tantalum, successively supplying

predetermined quantities of air to said tantalum while heating the tantalum to its air absorbing temperature until said tantalum absorbs the air supplied thereto in the proportion of about 1000 cubic centimeters of air to 1000 grams of tantalum, and continuing the heating of said tantalum with the air absorbed thereby to diffuse the air throughout the tantalum.

5. A method of hardening a hard refractory metal from the group consisting of tantalum and columbium by diffusing a regulated quantity of a constituent of air through said metal, which comprises degasifying said hard refractory metal by heating it at a reduced pressure to from 1200° to 1400° C., supplying a measured quantity of air to said hard refractory metal, heating said hard refractory metal to the absorbing temperature for a hardening constituent of air whereby to cause absorption of said hardening constituent in the measured quantity of air by said hard refractory metal, continuing such heating of said hard refractory metal to cause said constituent of air to penetrate into said hard refractory metal whereby to harden it throughout, and controlling the quantity of air supplied to said refractory metal whereby to control the hardness of the resulting product.

6. A method of hardening tantalum, which comprises heating tantalum to the degasification temperature thereof in a vessel while maintaining the atmosphere in said vessel at a pressure of about one millimeter of mercury to remove the occluded gases from the tantalum, and thereafter simultaneously supplying air to the vessel containing the tantalum and heating said tantalum to its air absorbing temperature to cause it to absorb the air so supplied thereto.

7. A method of hardening tantalum, which comprises heating tantalum to the degasification temperature thereof in a vessel while maintaining the atmosphere in said vessel at a pressure of about one millimeter of mercury to remove the occluded gases from the tantalum, thereafter simultaneously supplying air to the vessel containing the tantalum and heating said tantalum to its air absorbing temperature to cause it to absorb the air so supplied thereto, and dispersing the absorbed air throughout the tantalum by continuing the last mentioned heating step.

8. A hard article of manufacture, comprising tantalum and air, the air being substantially uniformly distributed throughout the tantalum in the proportion of about 1000 cubic centimeters of air to 1000 grams of tantalum.

9. An article of manufacture comprising a hard spinneret of tantalum and air, the air being substantially uniformly distributed throughout the tantalum in the proportion of about 1000 cubic centimeters of air to 1000 grams of tantalum.

10. A method of hardening a hard refractory metal from the group consisting of tantalum and columbium by diffusing a regulated quantity of air through said metal, which comprises heating the hard refractory metal to the degasification temperature thereof while maintaining a sub-atmospheric pressure to remove the occluded gases from the hard refractory metal, thereafter supplying sufficient air to produce a product of desired hardness when the air is absorbed by the hard refractory metal, and heating the hard refractory metal to its air absorbing temperature to cause it to absorb the air so supplied thereto.